

April 30, 1929.

F. SMITH

1,710,747

METHOD OF AND APPARATUS FOR COATING METAL

Filed Dec. 7, 1925



INVENTOR  
*Franklin Smith*  
BY  
*Sydney J. Prescott*  
ATTORNEY

## UNITED STATES PATENT OFFICE.

FRANKLIN SMITH, OF BROOKLYN, NEW YORK, ASSIGNOR TO AMERICAN MACHINE & FOUNDRY COMPANY, A CORPORATION OF NEW JERSEY.

## METHOD OF AND APPARATUS FOR COATING METAL.

Application filed December 7, 1925. Serial No. 73,877.

This invention involves a method of, and an apparatus for, coating metal with a non-corrosive metal, relating more particularly to the coating of ferric wire with lead.

5 The main object of the invention involves the utilization of condensation of hot metallic vapor on relatively cold metal, and/or the utilization of glow discharge to effect a bombardment of the metal or wire with

10 myriads of minute particles of lead or other protective metal. Another object of the invention is the production of a method of, and an apparatus for, coating metal by the use of these forces, in order that the coating

15 may be effected at a high rate of speed which has been heretofore unattainable, and at a greatly reduced cost of production. With these and other objects not specifically mentioned in view, the invention consists in cer-

20 tain acts and series of acts, and in certain apparatus, constructions, and combinations, which will be hereinafter fully described and then specifically set forth in the claims hereunto appended.

25 The figure in the drawing illustrates in section an apparatus constructed in accordance with the invention, and by means of which the method may be carried into effect. The invention involves as essential elements

30 a method of coating metal and an apparatus for carrying that method into effect. The method consists in the condensation of metallic vapor upon the metal object to be coated. This condensation may be effected

35 by temperature difference, or, preferably, by electric deposition of the vapor particles by means of the glow discharge. By the preferred method, the vapor particles in the neighborhood of the molten metal become ionized chiefly by glow discharge. The ions combine with or condense upon the vapor particles, dragging these with them to the object to be coated, which is of opposite polarity.

40 The velocity of the vapor particles is proportional to their charge and to the voltage gradient of the dielectric field between the molten metal and the object to be coated. To avoid the electrical insulation difficulties at the higher temperatures, the vapor pres-

45 sure is maintained at a pressure less than atmospheric.

In the best practice of the method, therefore, the self-depositive properties of the vapor are thereby so augmented that the

metal may be properly coated by passing it through the vapor as rapidly as it is practicable to handle it. The best practice of the method further contemplates sand-blasting, or otherwise cleaning, the metal immediately before it is immersed in the metallic vapor, or passed therethrough. When sand-blasting is employed, the air used tends to prevent ingress of air to the coating chamber which confines the atmosphere embracing metallic vapor at sub-normal pressure, by blowing the sand outwardly through the metal inlet of the chamber. And, similarly, when the coating is to be chilled, the air used tends to prevent ingress of air to the coating chamber, by blowing outwardly through the metal outlet of the chamber.

The method branch or essential element of the invention may be varied within the scope of the method claims; and the specific apparatus created for carrying the method into effect, and used to illustrate the invention, is but one of numerous possible concrete embodiments of the same. The invention, therefore, is not to be restricted to the precise details of the method and apparatus branches or essential elements of the invention shown and described.

The apparatus shown was especially created for coating ferric wire with lead; and it is provided with a coating chamber 1 having at its bottom an inlet 2 through which the wire to be coated is introduced into the chamber 1, and having at its top an outlet 3 through which the coated wire passes out of the apparatus. The coating chamber 1 is mainly in the form of a steel cylinder having a removable cover 4 at its top. Extending upwardly from the centre of this cover is a tube 5 which terminates at the outlet 3 before referred to. Extending downwardly from the centre of the bottom of the cylinder is an expansion tube 6 which terminates at the inlet 2 before referred to. In the operation of the apparatus, the wire to be coated passes upwardly through the inlet 2, the expansion tube 6, the centre of the cylinder forming the main part of the coating chamber 1, the tube 5, and the outlet 3.

Means are provided for producing in the coating chamber 1 an atmosphere embracing lead or other metallic vapor of a self-depositive nature. This vapor is produced by

the following instrumentalities: Suspended from the cover 4, by means of lead-ins 7, 8, is a melting pot 9 of annular form, the wire to be coated passing up through an aperture 10 at its centre. The pot 9 rests on a centrally-apertured disc 11 through which the lead-ins 7 and 8 pass. The pot 9 is surrounded by a heating coil 12 which is included in a low voltage circuit (6 volts) of high amperage, said circuit also including the lead-ins 7 and 8. The coil 12 heats the lead or other metal in the pot 9 to maintain the desired vapor pressure within the coating chamber 1. Surrounding the coil 12 is a heat shield 13 of graphite for preventing overheating of the coating chamber walls opposite the pot 9. The lead-ins 7 and 8 are supported by insulators 14, 14, screwed into the cover 4 before referred to. These insulators may be made of the well-known fused silica. Each is surrounded by a metallic tube 15 the purpose of which is the prevention of condensation of metallic vapor on the insulators which, if permitted, would short-circuit the apparatus and render it useless. The condensation of the metallic vapor is prevented by the dielectric fields between the lead-ins 7 and 8 and the tubes 15. One side of the high voltage circuit is grounded on the vacuum chamber 23 as indicated on the drawing; the insulated side enters the coating chamber 1 through the lead-in 7 which is insulated from ground by the insulator 14. Connection is made to the metal in the pot 9 through the heating coil 12, the lead-in 8 and pipe 19. The low voltage circuit, which obviously is insulated from ground for the voltage of the high voltage circuit, enters the coating chamber 1 through insulators 14—14 as clearly shown on the drawing.

As the lead or other metal in the pot 9 is converted into metallic vapor, the supply in the pot must be replenished from time to time. With this end in view, the upper part of the lead-in 8 is hollow and connected, by means of a pipe 16, with a filling receptacle 17 located in any convenient and operative position. The receptacle 17 and pipe 16 are kept hot by well-known means not shown. The hollow part of the lead-in 8 terminates at its lower end at a T 18 with which is connected a bent pipe 19 leading to the interior of the pot 9. When the pot 9 needs replenishing, molten metal is forced from the receptacle 17 through the pipe 16, T 18, and pipe 19, to the pot 9.

As has been indicated in the foregoing, the metallic vapor pressure in the coating chamber 1 is maintained at a pressure less than atmospheric. Means are provided therefor which include a suction duct 20 leading from the tube 5, before referred to, towards a suitable vacuum pump of well-known construction and operation and there-

fore not shown in the drawing. Air is exhausted from the vapor chamber 1 by this means until a pressure of approximately 10 inches of mercury is reached, or, in other words, until the pressure is approximately 70 20 inches below normal atmospheric pressure at sea level. And there it is maintained as constantly as possible.

In order to increase the efficiency of the apparatus, means are provided to prevent 75 water from entering the vacuum chamber 26 or the pump. With this end in view, there is provided a duct 21 connected with the expansion tube 6 at one end and to the dehydrating chamber 22 at the other end. A 80 similar dehydrating chamber 28 is connected to the vacuum chamber 26 by means of a duct 27. Each of these dehydrating chambers contain a suitable deliquescent salt, for example phosphorus pentoxide, indicated on 85 the drawing as 23. The outlets of these dehydrating chambers are indicated on the drawing by arrows and are connected to suitable pumps of well known construction and operation and not shown on the 90 drawing.

For the purpose of cleaning the wire immediately before it enters the coating chamber 1, there is provided means for sand-blasting it at the inlet 2. This sand-blast 95 means includes a suitable blower of well-known construction and operation and therefore not shown, and a sand-blast pipe 24 opening into the tube 6 near the inlet 2 in such manner as to blow outwardly through 100 the inlet 2, thus effectually cleaning the wire immediately before it enters the coating chamber 1 and insuring a clean surface for the reception of the lead or other metal coating. Moreover, this outgoing blast of 105 air and sand effectually prevents ingress of air through the inlet 2, thus preventing disturbance of the partial vacuum existing in the chamber 1.

For the purpose of cooling or chilling the 110 coating on the wire immediately after it has been applied, provision is made for a cooling blast of air blowing outwardly through the outlet 3 before referred to. This includes a bent pipe 25 so associated with the outlet 115 3 as to direct a blast of cool air out through said outlet with the wire, thereby cooling or chilling the coating on the latter. The air blast flowing through the pipe 25 is derived from a suitable blower of well-known construction and operation and therefore not shown. It prevents ingress of air, thus avoiding disturbance of the partial vacuum existing in the chamber 1.

Naturally, the coating chamber 1 must be 125 very hot, and in order to provide heat insulation for the same, the said coating chamber is surrounded by a vacuum chamber 26 wherein a vacuum as nearly perfect as possible is desirable. The dehydrating 130

chamber 28 is like the dehydrating chamber 22, and carries a like dehydrating agent.

For the purpose of cooling the tops of the coating chamber 1 and vacuum chamber 5 26, a series of water pipes 29 lie coiled about the upper surface of the coating chamber cover 4, and a similar series of water pipes 30 lie coiled about the upper surface of the vacuum chamber 26.

10 When coating by condensation alone, atmospheric pressure may be used, though low pressure results in more rapid condensation. The lower the pressure, the lower the temperature at which the method may be 15 worked. But when coating electrically, either alone or in conjunction with condensation, low pressure is essential, and the relative high voltage must be unidirectional. There is a choice of polarity, however, as a 20 better and more rapid deposit is obtained by cathodic bombardment; that is, when the metal to be coated is positive.

The operation of the apparatus is as follows: Assuming that the vacuum pumps 25 have been working long enough to produce a partial vacuum in the coating chamber 1, and a sufficiently low pressure in the vacuum chamber 26, and that the low voltage circuit including the heating coil 12 has been in 30 operation long enough to heat the lead or other metal in the pot 9 to the desired vapor pressure wire to be coated may then be led upwardly through the apparatus, as by wire already coated and married to its end for 35 this purpose. The incoming wire is thoroughly cleaned by the sand blast at the inlet, and when it reaches a point just above the melting pot 9, the difference of temperatures of the hot vapor and of the cold wire 40 results in condensation of vapor on the surface of the wire. By the preferred method, however, the metallic vapor is condensed on the metal to be coated by electrical deposition as has been indicated in the foregoing. 45 A unidirectional current of about 2,000 volts is employed, the energy of which is limited to prevent transition from glow to arc discharge. There is a choice of polarity as a 50 better and more rapid deposit is obtained by cathodic bombardment; that is, when the metal to be coated is positive. As the wire to be coated passes through the coating chamber, it will be bombarded by myriads of metallic vapor particles which rapidly condense upon the wire and form a relatively 55 thick and tenacious coating. The wire should be passed through the coating chamber as rapidly as it is mechanically practicable. As the coated wire emerges from the 60 outlet 3, the coating is chilled by the air blast hereinbefore described. Once started, the operation is continuous, so long as the supply of metal in the pot is maintained.

65 Stuffing boxes, of well-known construction and operation and therefore not shown, may

be used instead of the outgoing blasts at the inlet 2 and outlet 3, if desired.

Also, the tubes at the inlet 2 and outlet 3 may be approximately 20 feet long, in which case no stuffing boxes, and no outwardly-directed air-blasts, will be required merely to maintain the low pressure in the coating chamber, for the reason that such great lengths relative to the small diameters of 70 said inlet and outlet enables the pumps to maintain the low pressure in the coating chamber. Also, a smoothing die for the 75 coated wire, of well-known construction and operation and therefore not shown, may be used at the outlet 3, if desired.

What is claimed is:

1. The method of metallically coating metal, which consists in thermally vaporizing the coating metal, then ionizing the metallic vapor, and electrically depositing and 80 condensing the ionized vapor on the metal to be coated.

2. The method of metallically coating metal, which consists in thermally vaporizing the coating metal at sub-atmospheric 90 pressure, ionizing the metallic vapor, and electrically depositing and condensing the ionized vapor on the metal to be coated.

3. The method of metallically coating metal, which consists in thermally vaporizing the coating metal, ionizing the metallic vapor, cleaning the metal to be coated, and electrically depositing and condensing the 95 ionized vapor on the cleaned metal.

4. The method of metallically coating 100 metal, which consists in thermally vaporizing the coating metal, ionizing the metallic vapor, passing the metal to be coated through the ionized vapor, and electrically depositing and condensing the ionized vapor 105 on the passing metal.

5. The method of coating ferric wire with lead, which consists in thermally vaporizing the lead, ionizing the lead vapor, and electrically depositing and condensing the 110 ionized vapor on the wire.

6. An apparatus for coating metal, comprising a coating chamber, means for thermally vaporizing coating metal in said chamber, and means for ionizing and electrically depositing and condensing the ionized vapor on the metal to be coated in said 115 chamber.

7. An apparatus for coating metal, comprising a coating chamber, means for thermally vaporizing coating metal in said chamber, means for ionizing and electrically depositing and condensing the ionized vapor on the metal to be coated in said chamber, and means for cleaning the metal to be 120 coated as it enters said chamber.

8. An apparatus for coating metal, comprising a coating chamber, means for thermally vaporizing coating metal in said chamber, means for ionizing and electrically 125 depositing and condensing the ionized vapor on the metal to be coated in said chamber, and means for ionizing and electrically 130

depositing and condensing the ionized vapor on the metal to be coated in said chamber, and means for chilling the applied coating as the coated metal leaves said chamber.

5 9. An apparatus for coating metal, comprising a coating chamber, means for maintaining sub-atmospheric pressure in said chamber, means for thermally vaporizing coating metal in said chamber at said sub-  
10 atmospheric pressure, and means for ionizing and electrically depositing and condensing the ionized vapor on the metal to be coated in said chamber.

10 15. An apparatus for coating metal, comprising a coating chamber having an inlet at its bottom and an outlet at its top for the metal to be coated, means for thermally vaporizing coating metal in said chamber, and means for ionizing and electrically de-  
20 positing and condensing the ionized vapor on metal passing through said inlet, said chamber, and said outlet.

11. An apparatus for coating metal, comprising a coating chamber having an inlet at its bottom and an outlet at its top for the metal to be coated, means for thermally vaporizing coating metal in said chamber, means for ionizing and electrically deposit-  
25 ing and condensing the ionized vapor on metal passing through said inlet, said chamber, and said outlet, and means for cleaning the metal to be coated as it passes through said inlet.

12. An apparatus for coating metal, comprising a coating chamber, means for thermally vaporizing coating metal in said chamber, means for ionizing and electrically de-  
30 positing and condensing the ionized vapor on the metal to be coated in said chamber,  
40 and a suction duct leading from said chamber to establish therein sub-atmospheric pressure.

13. An apparatus for coating metal, comprising a coating chamber, means for thermally vaporizing coating metal in said chamber, means for ionizing and electrically de-  
45 positing and condensing the ionized vapor on the metal to be coated in said chamber, a suction duct leading from said chamber, and dehydrating means associated with said duct.

14. An apparatus for coating metal, comprising a coating chamber, means for thermally vaporizing coating metal in said chamber, means for ionizing and electrically de-  
55 positing and condensing the ionized vapor on the metal to be coated in said chamber, and a heat-insulating vacuum chamber surrounding said coating chamber.

15. An apparatus for coating metal, comprising a coating chamber, means for thermally vaporizing coating metal in said chamber, means for ionizing and electrically de-  
60 positing and condensing the ionized vapor on the metal to be coated in said chamber, a vacuum chamber surrounding said coating chamber, and means for cooling the tops of both chambers.

16. An apparatus for coating metal, comprising a coating chamber having an inlet and an outlet each of which is of great length relative to its diameter, means for thermally vaporizing coating metal in said chamber, and means for ionizing and electrically de-  
70 positing and condensing the ionized vapor on the metal to be coated in said chamber.

In testimony whereof, I have signed my name to this specification.

FRANKLIN SMITH.